

1

3,600,272

**POLYETHYLENEIMINE CURED  
EPOXY-MODIFIED PAPER**

Louis R. Cortigene, Portland, and William R. Sherman,  
Cape Elizabeth, Maine, assignors to Scott Paper Com-  
pany, Delaware County, Pa.  
No Drawing. Filed Aug. 29, 1968, Ser. No. 756,312  
Int. Cl. D21d 3/00; D21h 3/36

U.S. CL. 162—164

13 Claims

**ABSTRACT OF THE DISCLOSURE**

Process for producing epoxy-modified paper by a chemical reaction on a conventional paper machine by adding at separate points in the papermaking process upstream of a heating section a high molecular weight, polyethyleneimine which is substantive to paper and adding at a separate point an aqueous dispersion of an unreacted epoxy resin such as vinyl cyclohexane dioxide which is curable by said polyethyleneimine.

This invention relates to a process for making epoxy-modified paper, and to the product of the process. The process is performed on a conventional paper machine in the sections of the paper machine upstream of a heating section and involves the application to the paper of a high molecular weight, polymeric material which is substantive to paper, and the incorporation at a separate step of an aqueous dispersion of an unreacted epoxy resin which is curable by said polymer. The invention is also directed to the epoxy-modified papers of improved properties which are produced by the application of the aforesaid process.

In the conventional formation of paper, paper strength is achieved by the hydrogen bonding which occurs between contiguous fibrils of individual paper fibers. These bonds, although adequate to maintain the integrity of the paper sheet, are not strong enough to provide paper with high strength and abrasion resistance properties. Consequently, paper is ordinarily used for those low-strength-requirement applications in which its cost of manufacture relative to available substitutes, such as plastic sheeting or non-woven fibers, is low. This low cost is due to the low cost of the wood pulp used in producing paper, and the extremely high machine speeds, as high as 5000 linear feet per minute on tissue-making machines, with which paper is capable of being produced.

The strength of paper can be improved by the incorporation of certain additives, and to this end so-called wet strength resins, such as urea formaldehyde and melamine-formaldehyde resins, are often incorporated in paper to maintain the strength of the paper in circumstances in which paper is submerged in water. Also, in the printing and converting field, in which paper is produced for reproduction applications, such as typing paper, or to be converted into tabulating card stock or the like, starch or other sizing compounds are often incorporated in paper in order to increase the strength, stiffness, abrasion, resistance, and similar physical properties thereof.

For certain applications, such as tabulating card stock, these conventional strength-increasing techniques are insufficient to produce a paper which will satisfactorily withstand the extreme conditions of use to which the paper is subjected. For example, a tabulating card which must be printed, punched, and frequently run many times through a computer feed mechanism, takes a considerable physical beating. Any disfigurement of the tabulating card can result in costly, time-consuming, machine jamming which encumbers the very high speed computer operation process. Of course, the familiar legend "do not fold,

2

spindle or mutilate," is utilized to minimize these machine feed problems. On the other hand, with constant use, abrasion, corner folding and other wear phenomena occur on the individual tabulating cards which result in card feeding mechanisms becoming jammed. It is therefore most desirable to be able to provide a relatively inexpensive technique for improving the wear properties of such tabulating card stock.

In U.S. Pat. No. 3,131,083, there is disclosed a process 10 for impregnating tabulating card stock with certain epoxy resins and their curing agents. These resins are applied in an "off the machine" process, as a separate and distinct operation from the ordinary formation of the paper sheet. In the process of the aforesaid patent, a tabulating card 15 stock paper sheet would be produced on a conventional paper machine, and the untreated end product would be wound on a so-called parent roll. The thus-formed paper from the parent roll would then be subjected to the after-treatment described in the 3,131,083 patent. The resin and curing agent would be applied from an organic solvent, which is used to disperse and distribute the resin, and, after impregnating the paper with the resin, curing agent, and solvent, the impregnated paper is heated to 20 volatilize the solvent, leaving a residue of cured resin 25 impregnating the paper. Because of the necessity for removing virtually all solvent in the paper, the paper treated pursuant to said process is heated to such an extent that the moisture content of the paper is reduced below minimum acceptable standards for adequate performance of 30 the paper. Consequently, after the paper has been treated with the solvent system and dried, the paper must be rewetted to raise its moisture content to the minimum acceptable level. Furthermore, the process of said Pat. 3,131,083 does not provide any significant chemical linking 35 between the epoxy resin and the paper fibers, but rather results in the paper fibers being mechanically imbedded in the cured resin. The foregoing prior art process is, therefore, expensive because of the necessity for an "off the machine" process with separate moisture 40 addition, and because of the elaborate safety precautions which must be utilized when handling organic solvents, in order to obtain proper removal of the solvents from the ambient, to prevent a hazardous working condition for those employees working in the coating operation. 45 Too, because of the mechanical nature of the epoxy paper bond physical properties are not optimized.

The instant invention overcomes the foregoing disadvantages of the above-noted prior art processes, by providing a process which can be utilized on a conventional paper machine, without any change of the operating speeds and conditions of the paper machine, utilizing only equipment which is available on many conventional paper machines. Therefore the necessity for a separate, off-machine coating process and coating equipment is 50 avoided. Also, because no solvents are used, no safety hazard is presented. Moreover, in the practice of the instant process, epoxy resin cure occurs during the formation of the paper and the formation of the hydrogen bonds, and the epoxy resin itself participates in polymerization 55 with the paper fibers to provide chemical, as well as mechanical, bonds with the paper fibers, to provide increased strength and improved physical properties of the end product.

Because the process of this invention significantly improves 60 the tensile strength and wet rub resistance as well as other physical properties of paper produced thereby, this process represents a technique for utilizing a paper machine for the production of materials which may be used as textile substitutes. In evaluating the applicability 65 of paper as a textile substitute, for such uses as paper clothing, paper towels, paper bedding, and the like, the tensile and wet strength limitations of conventional paper

have been significant shortcomings. So-called sanitary papers, such as are used in the formation of paper napkins, toilet tissue, and facial tissue, are capable of providing an acceptable softness and drape to render these materials useable as textile substitutes. However, their physical properties are such that they are not satisfactory substitutes. Also, because of the relatively weak bonding between fibers, they are more difficult to satisfactorily print, because of fibers leaving the paper and adhering to the printing plate. Conventional paper strength improvement techniques have been inadequate to overcome these shortcomings, because of inadequate strength improvement, and since some of the techniques for improving the physical properties of paper render the paper stiff and hard and therefore unsuitable for use as a textile substitute.

The instant process overcomes these foregoing disadvantages of the prior art by providing a relatively economical technique for improving the physical properties of the soft, drapable, low strength, sanitary papers while retaining the softness and drapability normally inherent in such papers.

Since the instant process produces paper products which have increased strength, including abrasion resistance, tensile strength, and the like, the process may be utilized in the entire spectrum of paper products for the purpose of improving the physical characteristics of these products when the performance demands are adequate to justify the added cost of the materials required by this process.

The process of the instant invention requires that an uncured epoxy resin which is capable of being dispersed in water, and a high molecular weight, polymeric material which functions to initiate polymerization of the epoxy resin, i.e. serves as a curing agent for the resin, be applied to the paper being formed in discrete applications, prior to the heating of the paper in a dryer section of the paper machine. It should be noted that in conventional paper machines drying is accomplished in the press section as well as in the heating section. In the press section water is removed to some extent by evaporation, to some extent by wicking, and to some extent by gravity flow. However, for purposes of this patent application the dryer section of the paper machine is defined to include only that section of the machine in which one or more heated rolls are used for the purpose of evaporating some of the water in the paper.

It should also be understood that, although some paper machines may be used for the application of the instant process without modification, the variations between individual paper machines are great, and specific machines might have to be modified to permit the most economical use of the process. For example, paper machines which are solely or primarily used for the production of the so-called sanitary papers will not conventionally include a size press, because size is not added to these papers, and a size press might have to be added to a sanitary paper machine for the practice of this process.

Generally, the instant process contemplates the addition to the paper, preferably at the size press of an aqueous dispersion of an uncured, water dispersible epoxy resin which is readily curable, and the discrete introduction of a water dispersible, high molecular weight, polymeric curing agent for the unreacted epoxy resin, which curing agent is substantive to paper. The polymeric curing agent is preferably added to the paper before the epoxy resin dispersion is added, and is most preferable present in the furnish.

It is therefore an object of this invention to provide a process which may be applied on a conventional paper machine, often without any modification of the paper machine per se or of its operating conditions, to improve the physical properties of the paper, particularly, tensile

strength, abrasion resistance, fold endurance and delamination resistance.

Another object of this invention is to provide a process for making paper having improved internal bond strength.

It is an additional object of this invention to provide a paper product which has improved physical properties, particularly tensile strength, abrasion resistance, and fold endurance.

Another object of the invention is to provide a process for producing an improved tabulating card stock, useable on a conventional machine for producing such card stock, and providing a tabulating card having improved durability, abrasion resistance, delamination resistance, tensile strength, fold endurance, and nick resistance.

Yet another object of this invention is to produce a paper product which has the softness and drapability of textiles, and also has a tensile and abrasion resistance which is superior to ordinary paper, and which is useable as a textile substitute.

A concomitant object of this invention is to provide a process for producing an epoxy-modified paper by the addition to the furnish of a high molecular weight, paper substantive, polymeric epoxy curing agent, and by the addition at a discrete point in the papermaking process upstream of a dryer section, and preferably at the size press, of an aqueous dispersion of a low molecular weight uncured epoxy resin which is heat curable at relatively low temperatures.

It is to be noted that conventional paper machines operate at extremely high machine speeds. Machines for the production of printing papers will operate at speeds in the range from about 500 to about 2000 linear feet per minute, and machines for the production of sanitary papers, such as facial tissue paper, will frequently operate at machine speeds in the range from about 2000 to about 5000 feet per minute. Although the length and residence time of a sheet of paper in a dryer section of the paper machine will vary significantly, generally a sheet of paper will have a residence time ranging between about  $\frac{1}{10}$  of a second and about 5 seconds in a dryer section of a paper machine. The shorter residence times are those which exist on the high speed sanitary paper machines, wherein most or all of the heating is accomplished by a single heated shell which may be 15 feet in diameter, and is referred to in the art as a "Yankee dryer." A Yankee dryer may or may not have upstream or downstream auxiliary heaters depending on the specifics of the particular paper machine in question.

In manufacturing printing and converting papers, Yankee dryers are not usually utilized, and the dryer section of a machine for making printed and converting papers, such as tabulating stock may often incorporate between about 40 and about 70 dryer units, which are heated shells having a diameter which may be in the range from about 2 $\frac{1}{2}$  to about 6 feet. Dryers may be located at a number of different places on a paper machine, such as in the conventional dryer section, at the calender stacks or downstream of the calender stacks, and the process of this invention may be applied before any of those dryers.

Although, in the paper industry, the temperature at which the paper being heated will vary substantially, depending on the nature of the specific machine being considered, generally, paper being heated on an ordinary paper machine will be subjected to a temperature in the range from about 170° F. to about 220° F., although in some instances, on the very large, high speed machines, temperatures as high as 250° F. or 300° F. may be encountered.

One step of the process of this invention is the addition to the paper being formed of an aqueous dispersion of a relatively low molecular weight, epoxy resin. The epoxy resins utilized will have a molecular weight of about 1000 or less, and most preferably the epoxy resins utilized will have a molecular weight of 500 or less, and have two or

more epoxy units, an epoxy unit being defined as a moiety in which an oxygen atom is connected to two adjacent carbon atoms whereby the oxygen atoms may react with active hydrogen groups. The unreacted epoxy resins of choice will have a molecular weight of 500 or less, and be polyepoxides containing two or more epoxy groups per molecule. These epoxy resins will be dispersible in water, and will be relatively highly reactive, so that addition of a curing agent to the resin will produce cure or polymerization of the unreacted epoxy resin at a relatively high rate, without the necessity for the addition of excessive amounts of heat.

Because of the high machine speeds and relatively low operating temperatures on paper machines the uncured epoxy resins utilized in this invention are substantially completely curable in a relatively short period of time, because of the short time during which the paper is on the paper machine, and the even shorter time during which the paper is passing through a dryer section, and due to the relatively low temperatures present in the dryer sections. The uncured epoxy resins having molecular weights under about 1000, and particularly such resins having molecular weights of about 500 or less, are often quite reactive, because of their short chain length per unit weight, and are readily dispersed in aqueous media. Also, these low molecular weight resins are of relatively low viscosity, and in order to get acceptable application of the resin, the viscosity of the aqueous dispersion containing the epoxy resin must be low enough to permit good penetration of the resin into the paper. Maximum tolerable viscosity will vary, depending upon the particulars of the paper machine in question and its conditions of operation. It is preferred that the viscosity of the epoxy dispersion be 100 centipoises or less at 25° C.

Frequently it will be most convenient to apply the epoxy to the paper at the size press as part of the size solution. In such instances the size solutions may also contain starch, which is conveniently used as a size material, and the viscosity of the individual resin or resins, the starch, water, and other surfactants as an entity will be no more than 100 centipoises, and will most preferably be as low as possible. It is desirable to keep the viscosity of the epoxy dispersion as low as possible, when the epoxy is added to already formed paper, as when the epoxy is applied to the paper downstream of the wire. This is important because the lower the viscosity of the dispersion, the more readily the resin dispersion may be wicked into the paper to obtain uniform distribution of the epoxy resin throughout the cross-section of the paper; therefore optimum properties of the epoxy-modified end product are obtained because the paper is thoroughly impregnated with resin to produce good chemical bonding of the epoxy resin and paper fibers throughout the cross-section of the paper.

As has been well described in the prior art, there are enumerable epoxy resins which are presently commercially available. Of those resins any uncured epoxy resin having a molecular weight of about 1000 or less may be used which is water dispersible, cure of which may be initiated by a cellulose substantive, high molecular weight polymer, and the reactivity of which is such that its cure may be substantially effected by heating at temperatures in the range from about 150 to about 220° F. for relatively short periods of time on the order of one-fifth of a second to ten seconds. The most preferred resins are those which have a molecular weight of about 500 or less because these are most reactive in relation to their weight, and because dispersions of these resins have low viscosity. In this regard some preferred epoxy resins are vinyl cyclohexane dioxide, alicyclic diepoxy carboxylate and 1,4-butanediol diglycidyl ether. The epoxy resin will preferably be present in an amount in the range from about 0.1% to about 30% by weight of the aqueous dispersion.

This aqueous dispersion of uncured epoxy resin may include any amount of a papermakers starch which can

be used as a paper size. The starch thickens the dispersion, and makes the particles of the epoxy emulsion more readily supported, and therefore prevents these particles from coming out of dispersion. The amount of resin and starch will preferably be adjusted so that at no time is the viscosity of the dispersion of resin greater than about 100 centipoises. As noted above, it is most preferable that the viscosity of the aqueous dispersion of resin be as much below 100 as reasonably practicable. It is preferred that the amount of epoxy resin be in the range of about 2 to about 12% by weight of the total aqueous dispersion, and the most preferred amount of resin is from 2% to 8%. Although any papermaking starch can be added to the resin dispersion, a particularly useful starch in the manufacture of tabulating card stock is Penford Gum 380, which is an hydroxyethylated starch.

The epoxy dispersion may include two or more unreacted epoxy resins. It is necessary that one of these epoxy resins be an unreacted polyepoxidized resin, having a molecular weight of about 500 or less. The other resin or resins, the amount of which will usually be no more than equal to the amount of the low molecular weight resin, may be one or more unreacted polyepoxides having a molecular weight less than 1000. The higher molecular weight resin must be water dispersible without the use of an organic solvent in order that a completely aqueous system may be maintained. Additionally, it is necessary to balance the amount of the uncured epoxy resins present, so that the viscosity of the resin dispersion may be maintained as low as possible, and generally below about 100 centipoises, and so that the reactivity of the higher molecular weight resin or resins is sufficiently fast that the resin may be substantially completely cured on the paper machine. Some suitable higher molecular weight polyepoxide resins are the bisphenol A-epichlorohydrin type of resins having molecular weights less than 1000. The higher molecular weight epoxy resin should also be curable by the curing agent for the other resin.

It may be desired to facilitate and maintain the dispersion of the resin in water by use of an emulsifying agent. These emulsifying agents are surfactants or wetting agents, and are well-known in the art. Some suitable such surfactants are mono- and di-glycerides from the glycerolysis of eatable fats, polyoxyethylene, sorbitan, fatty acid esters such as polyoxyethylene sorbitan monolaurate, polyoxyethylene sorbitan monopalmitate, polyoxyethylene sorbitan monostearate, polyoxyethylene sorbitan tristearate and polyoxyethylene sorbitan monooleate. The polyoxyethylene sorbitol esters, such as polyoxyethylene sorbitol oleate, polyoxyethylene sorbitol laurate and polyoxyethylene sorbitol tall oil may be also utilized. The polyoxyethylene alcohols, such as polyoxyethylene lauryl ether, polyoxyethylene cetyl ether, and polyoxyethylene stearyl ether may be utilized too. Combinations of one or more surfactants may also be used to disperse the epoxy resin. The amount of surfactant used will be in the range from about 0% by weight to about 10% by weight of the uncured epoxy resin in the aqueous dispersion.

It is to be noted that the aqueous dispersion of resin may also include other conventional size press additives, in addition to starch, so long as the cure of the resin is substantially unaffected, and the viscosity of the dispersion remains workable, preferably below about 100 centipoises. Some resins are curable only in a basic environment, some are only curable in an acid environment and some are only cured in a neutral environment. Thus, control should be exercised over the over-all pH of the paper during the course of the process, including the pH of any additives, so as not to prevent cure of the epoxy resin. The resins which are most preferred to be used in this invention, namely 1,4-butanediol diglycidyl ether and vinyl-cyclohexane dioxide are basic cured resins, and consequently such acid beater additives as rosin, which is abietic acid, and alum, another beater additive, are to be avoided.

Because the most preferred epoxy resins are curable in basic systems, the most preferred curing agents are the basic curing agents. In this regard, the most preferred curing agents are the cellulose substantive, high molecular weight, polymeric amines. By high molecular weight is meant those polymers having a molecular weight of about 500 or more, preferably a molecular weight of about 1000 or more, and most preferably a molecular weight in the range between about 20,000 and about 80,000. A particularly useful group of basic curing agents are the polyalkylene imines, such as polyethylene imine, polypropylene imine, poly-(2-methyl ethylene imine), and the like. Polyethylene imine is the most preferred curing agent, and this polymer is available in molecular weights ranging between about 500 and about 100,000. The most preferred curing agent is a polyethylene imine having an average molecular weight in the range between about 40,000 and about 60,000. One such polymer is commercially available under the trademark Tydex 12, and is a product of the Dow Chemical Company. Other substantially linear polymeric amines which are substantive to cellulose and have molecular weights substantially in excess of about 500 may be utilized, such as urea formaldehyde resins of the sort described in U.S. Pat. No. 3,275,605 and melamine-formaldehyde resins of the sort described in U.S. Pat. No. 2,345,543. The polyether diamines, having the general formula



may also be utilized, provided that the minimum molecular weight criterion is satisfied.

If a melamine-formaldehyde or a urea formaldehyde curing agent is utilized, the pH of the furnish must be maintained at 5.5 or less in order to prevent the curing agent from dropping out of solution, and in order to maintain the substantivity of the curing agent to cellulose.

The polymeric curing agent may be added at any point in the papermaking process prior to a dryer section, but it is most preferred that the curing agent be added upstream of the addition of the epoxy dispersion, and it is particularly desirable that the curing agent be present in the headbox. The curing agent may thus be added to the beater, the beater stock chest, and fan pump or may be introduced directly into the headbox. Any of these places for curing agent introduction prior to the headbox slice represents a convenient place for introducing the curing agent while insuring that the curing agent will be intimately and uniformly distributed throughout the furnish.

The curing agent may be present in an amount in the range from about 0.1% to about 10%, based upon the weight of the pulp (bone dry) in the furnish, and will preferably be present in an amount in the range from about 0.5% to about 4% of the pulp weight. Of course, the optimum amount of curing agent will necessarily be sufficient to initiate an effective degree of cure of the epoxy resin or resins within a relatively short period of time on the paper machine, so that the paper may be handled, as being rolled up, without blocking, and so that no substantial amounts of uncured resin are vaporized by the heat of the paper machine drying rolls.

As previously noted, it is preferable that basic curing resins be utilized, in which case the amine curing agents are the most desirable, and in those cases, the pH of the furnish will desirably be 7 or more, and will preferably be in the range between about 7.5 and about 10.

As noted above, the curing agents to be utilized in the instant process are those which are substantive to cellulose, that is to say those curing agents which are cationic in aqueous dispersion. The paper fibers, in aqueous dispersion, bear a negative electrical charge, and the cationic curing agents therefore are held to the paper fibers by secondary bonds. The relatively high molecular weight, i.e. 500 or more, curing agents will readily bridge two or more fibers, and because of the manner in which the curing agents participate in the polymerization of the

epoxy resin, these long chain curing agents contribute to the substantially improved strength qualities of the product of the instant process. If, as is most preferably the case, the high molecular weight, cationic, amine polymers are used as curing agents, particularly if a compound such as polyethylene imine having a 40,000 to 60,000 molecular weight, the curing agent, because of its cationic, cellulose substantive nature, will form a secondary chemical bond with a contiguous cellulose fiber. By virtue of the length of the curing agent polymer, it will physically contact and bond to two or more proximate cellulose fibers, and form a backbone for the formation of an epoxy polymer linking the fibers. The substantive polymeric amines, which are attached to the cellulose fibers, function, by virtue of the amine moieties thereof, as cross-linking agents, and as catalysts, for the polymerization of the uncured epoxy resin. Therefore, the amine curing agents, in performing their cross-linking function, will become a part of the epoxy polymer as well as functioning to catalyze polymerization thereof. Consequently, use of the high molecular weight polymeric curing agents significantly contributes to the improved properties of the paper.

Further contributions to the improved qualities of the product of the instant process are believed to be made by virtue of the epoxy resin and its curing agent contacting the cellulose fibers prior to substantial drying of the fibers and while hydrogen bonding of the fibers is incomplete. Under these conditions polymerization of the epoxy can occur at a point in which hydrogen bonding at the intersection of contiguous fibers is not yet complete, and the individual cellulose fibers can become a part of the epoxy polymer, thereby being bound to, and incorporated as part of the epoxy polymer by strong chemical bonds. Additionally, as the paper sheet dries after the aqueous dispersion of uncured epoxy resin has been added, a wicking action will occur with respect to the cellulose fibers which will cause the water and polymerizing epoxy resin to be drawn along the fibers to the fiber junctures. It is at these junctures of contiguous fibers that bonding of the fibers takes place, and as the paper dries the accumulation by this wicking action of polymerizing resin at the fiber junctures permits substantial amounts of the epoxy polymers to be concentrated at these junctures; this provides for increased paper strength due to the presence of the epoxy polymer at the place where additional strength is most needed and most useful, namely the fiber junctures. Thus, additional strength is provided in two ways, namely the mechanical incorporation of fiber junctions within the polymer as it cures, and secondly, the participation of the cellulose fibers in the polymerization reaction to provide a chemical bond between the cellulose and the epoxy polymer.

In its most preferred mode of application the process includes the incorporation of an amount of polyethylene imine having molecular weights in the range of about 40,000 and about 60,000 of 0.5% to 4%, based on the weight of the bone dry pulp. This curing agent is incorporated into the furnish by direct introduction thereof into the headbox. The furnish would not include any rosin, alum, or other acidic material, so that the pH of the furnish would be 7 or more. The curing agent could also be added to the paper at any other point downstream of the slice and upstream of a dryer section, by such means as spraying an aqueous solution of the curing agent on to the paper, adding an aqueous solution of the curing agent at the size press or any other similar techniques for intimately distributing the curing agent throughout the cross-section of the paper. When the curing agent is added to the furnish, the paper is formed into a web, as is usually the case, on a Fourdrinier wire, passes between suction boxes, over a couch roll, and into the press section, wherein further water is removed by pressing and by absorption by the felts. Downstream from the press section there is located a size press, which may be used for the introduc-

tion of an aqueous dispersion of the uncured epoxy resin to be incorporated in the paper. Most preferably, the size is an aqueous dispersion made up of about 2% by weight of 1,4-butanediol diglycidyl ether and 2% by weight of a bisphenol A-epichlorohydrin resin having a molecular weight of approximately 500. A surfactant or surfactants, such as a polyoxyethylene oleyl ether and a polyoxyethylene sorbitan monopalmitate, may be included in the aqueous dispersion in a total amount of about 1% of the weight of epoxy resin. The size may also include approximately 12% by weight of Penford Gum 380, hydroxyethylated starch. This aqueous dispersion would be applied at the size press, immediately after which the epoxy resin impregnated paper would proceed into a dryer section where it would be heated at a temperature in the range between about 180° F. and 210° F. for a period of about 2 to 4 seconds. Upon exit from the dryer section the sheet may optionally pass through one or more calender stacks, where it is calendered, may then pass over more dryers, and is finally wound up on a windup stand.

Although, in machines containing one or more size presses, it is preferred to add the uncured epoxy resin dispersion at the size press, the epoxy resin can be added at other points in the formation of the paper upstream of the dryer section, by such means as presses, spraying, and the like. The preferred sequence of introduction of the curing agent and the epoxy resin is that the curing agent be introduced into the paper first, and that the epoxy resin be introduced after the curing agent is uniformly distributed through the cross-section of the sheet. This sequence can be reversed, and it is within the purview of this invention to introduce the uncured epoxy resin first. However, the results achieved by initial introduction of the curing agent into the paper are superior; and the curing agent first, epoxy resin second, sequence is to be preferred.

Although papers are usually formed with wood fibers, it is within the contemplation of this invention that the furnish include in whole or in part other cellulosic fibers such as bagasse, jute, hemp, and rag fibers. The wood pulp fibers utilized in the process may be sulfite, kraft, soda, semi-chemical, and ground wood pulps as well as mixtures thereof.

The following examples are given as illustrative of the instant invention without, however, limiting the invention to the specific details of the examples.

#### EXAMPLE I

This example, as well as succeeding Examples II through XI, were run on an 18" paper machine, in most cases using a furnish of 67% pine and 33% hardwood. The furnish generally had a Canadian freeness of about 530, and included 3% by weight (based on the weight of the pulp on a bone dry basis) of Tydex 12, a polyethylene imine having a molecular weight ranging from about 40,000 to about 60,000. Tydex 12 is made by Dow Chemical Company.

The epoxy resin was added at the horizontal size press of the paper machine. In this example, the size was an aqueous solution containing 12% by weight of Penford Gum 380, a papermaking starch, and 20% by weight of Ciba's Araldite RD2, which is 1,4-butanediol diglycidyl ether.

The average machine speed was 155 feet per minute. The average temperature in the drying section was about 220° F.

The paper end product of this example had a basis weight of 107.7 pounds per 3,000 square foot ream and a caliper of 7.6 mils. The physical properties of the paper are set forth in Table I.

#### EXAMPLE II

A paper was made in the manner and under the conditions set forth in Example I, except that the size contained 6% by weight of PG 380 and 10% by weight of RD2 epoxy resin, rather than 20%. The product had a basis

weight of 104.9 pounds per ream and a caliper of 7.5 mils.

#### EXAMPLE III

A paper was made in the manner and under the conditions set forth in Example I, except that the size contained 12% by weight of Penford Gum 380, 10% of RD2, 10% of 6020, a bisphenol A-epichlorohydrin resin having a molecular weight of about 400, made by Ciba, and about 0.5% by weight, based on the resin weight, of each of Brij 92 and Tween 40. The product had a basis weight of 107.1 pounds per ream and a caliper of about 7.6 mils.

#### EXAMPLE IV

A paper was made in the manner and under the conditions set forth in Example I, except that the size contained 12% by weight of Penford Gum 380 and 6% of RD4, which is Ciba's vinylcyclohexene dioxide. The product had a basis weight of 98.8 and a caliper of about 7.4 mils. In this example, the furnish also included 0.25% by weight of each of sodium bicarbonate and Aquapel 360, an alkylketene dimer.

#### EXAMPLE V

A paper was made in the manner and under the conditions set forth in Example I, except that the size contained 12% by weight of Penford Gum 380 and 6% by weight of Ciba's CY 179, an alicyclic diepoxy carboxylate. The product had a basis weight of 102.2 and a caliper of 7.6 mils. In this example, the furnish also included 0.25% by weight of each of sodium bicarbonate and Aquapel 360.

#### EXAMPLE VI

A paper was made in the manner and under the conditions set forth in Example I, except that the size contained 10% by weight of Penford Gum 380, 2% of RD2 and 2% of 6020. The product had a basis weight of 104.3 and a caliper of 7.7 mils.

#### EXAMPLE VII

A paper was made in the manner and under the conditions set forth in Example I, except that the size contained 10% by weight of Penford Gum 380, 2% each of RD2 and 6020, and 1% each based on the weight of resin of two surfactants, Tween 40, a polyoxyethylene sorbitan monopalmitate of Atlas Ind., Inc., and Brij 92, a polyoxyethylene oleyl ether of Atlas. 2% of Tydex 12 polyethylene imine was used in the furnish, with no other furnish additives.

#### EXAMPLE VIII

A paper was made in the manner and under the conditions set forth in Example I, except that the size contained 10% by weight of a Penford Gum 380, 2% each of RD2 and 6020, and 0.8% by weight, based on the weight of the epoxy resins, of each of Brij 92 and Tween 40. The furnish contained 3% by weight of a urea formaldehyde resin, based on the weight of the wood pulp on a bone dry basis. The urea formaldehyde resin was manufactured in accordance with U.S. Pat. 3,275,605. The product had a basis weight of 96.6 and a caliper of 7.3 mils.

#### EXAMPLE IX

A paper was made in the manner and under the conditions set forth in Example I, except that the size contained 10% Penford Gum 380, 2% of RD2, 2% of 6020, and 0.7% each, based on the weight of the epoxy resins, of Brij 92 and Tween 40. The furnish contained 1.5% each by weight, based on the weight of the pulp on a bone dry basis, of a melamine formaldehyde resin prepared in the manner set forth in U.S. Pat. No. 2,345,543, and Tydex 12. The product had a basis weight of 107.7 and a caliper of 6.6 mils.

#### EXAMPLE X

A paper was made in the manner and under the conditions set forth in Example I, except that the size contained

## 11

10% Penford Gum 380, and 4% each of Epoxy 7, an aliphatic glycidyl ether, and 6020. The furnish was 85% sulfite and 15% kraft, having a Canadian Freeness of 530 and contained 3% of Tydex 12. The product had a basis weight of 101.8 and a caliper of 6.8 mils.

## EXAMPLE XI

A paper was made in the manner and under the conditions set forth in Example I, except that the size contained 10% Penford Gum 380, 4% of 6004, a low molecular weight bisphenol A-epichlorohydrin resin 4% of RD4 and 0.8% each, based on the weight of epoxy resin, of Tween 40 and Brij 92 surfactants. The furnish was 75% sulfite and 25% kraft, and included 1/2% alum, 3% melamine formaldehyde and  $H_2SO_4$  in an amount to adjust the pH of the furnish to 5.0. The furnish freeness was about 528. The product had a basis weight of 105.6 and a caliper of 6.8 mils. Table I shows the physical properties of the products produced by the respective processes of Examples I to XI inclusive.

## 12

molecular weight polymeric curing agents and various low molecular weight unreacted epoxy resins, in relation to the use of the curing agents per se, untreated paper, and non-polymeric curing agent used with a low molecular weight unreacted epoxy resin.

5 Examples (a) through (f) of Table III were produced by sequentially impregnating bench sheets with an aqueous solution of curing agent, removing excess moisture and curing agent, adding an aqueous dispersion of epoxy resin (where applicable) and curing at 220° F. In Example (f) the sequence was reversed and bench sheets were first impregnated with an aqueous dispersion of resin, excess moisture and resin were removed, an aqueous solution of curing agent was added and the sheets dried and 10 cured at 220° F.

15 Example (a) shows that the bonding in a sheet of paper can be improved by the addition of polyethyleneimine since the dry tensile and wet tensile were both improved. This ability of polyethyleneimine is well known in the 20 papermaking art.

TABLE I

|                            | EXAMPLE |      |      |      |      |      |      |      |      |      |      |
|----------------------------|---------|------|------|------|------|------|------|------|------|------|------|
|                            | I       | II   | III  | IV   | V    | VI   | VII  | VIII | IX   | X    | XI   |
| Mullen (p.s.i.)            | 92      | 70   | 82   | 70   | 74   | 103  | 105  | 95   | 75   | 73   | 75   |
| Tensile, M.D. (p.p.i.)     | 59.5    | 64.1 | 56.9 | 54.0 | 57.6 | 72.9 | 66.0 | 60.4 | 50.2 | 67.0 | 67.3 |
| Tensile, C.D. (p.p.i.)     | 42.2    | 37.9 | 43.1 | 35.4 | 33.2 | 41.9 | 37.6 | 33.6 | 35.6 | 34.8 | 36.2 |
| Wet tensile, M.D. (p.p.i.) | 17.8    | 17.3 | 16.7 | 9.9  | 12.0 | 12.7 | 13.5 | 9.6  | 12.1 | 12.9 | 14.0 |
| Wet tensile, C.D. (p.p.i.) | 10      | 10.9 | 9.5  | 6.9  | 6.6  | 7.4  | 7.2  | 5.8  | 6.9  | 7.0  | 7.6  |
| Taber stiffness, M.D.      | 16.0    | 17.3 | 18.3 | 17.2 | 17.5 | 24.5 | 18.9 | 17.6 | 18.9 | 20.2 | 21.1 |
| Taber stiffness, C.D.      | 9.0     | 8.0  | 10.3 | 8.7  | 7.8  | 11.1 | 9.3  | 9.2  | 7.5  | 8.2  | 10.5 |
| Porosity (sec.), 100 cc.   | 44      | 28   | 23   | 18   | 19   | 13   | 11   | 24   | 45   | 99   | 179  |
| M.I.T. fold, M.D.          | 775     | 534  | 293  | 228  | 177  | 551  | 641  | 920  | 626  | 261  | 450  |
| M.I.T. fold, C.D.          | 615     | 310  | 245  | 158  | 161  | 409  | 522  | 566  | 643  | 232  | 305  |
| M.I.T. aged fold, M.D.     | 3       | 32   | 40   | 32   | 49   | 251  | 317  | 314  | 290  | 141  | 168  |
| M.I.T. aged fold, C.D.     | 3       | 42   | 69   | 38   | 103  | 272  | 332  | 604  | 265  | 117  | 193  |

## EXAMPLE XII

A paper was produced on a commercial paper machine at a machine speed of 800 feet per minute. The furnish contained 3% of Tydex 12 by weight, based on the weight of the pulp. The Tydex 12 was fed in at the headbox fan pump. No rosin or alum were in the furnish.

The size press solution consisted of an aqueous dispersion of 10% by weight of P.G. 380, 3% of RD2, 3% of 6020 and 0.5% of each of Brij 92 and Tween 40, based on the resin weight.

Table II presents a comparison of the average physical properties of papers produced in a series of commercial runs as set forth above, a conventional commercial card stock which has not been epoxy-modified, and a commercial epoxy impregnated card stock produced by a process such as that described in U.S. Pat. 3,131,083.

TABLE II

|                            | Prior art epoxy<br>impregnated<br>card stock | Example<br>XII |
|----------------------------|----------------------------------------------|----------------|
| Basis weight               | 100                                          | 101            |
| Caliper (mils)             | 7.0                                          | 7.1            |
| Mullen (p.p.i.)            | 70                                           | 105            |
| Tensile, M.D. (p.s.i.)     | 63                                           | 66             |
| Tensile, C.D. (p.p.i.)     | 37                                           | 50             |
| Wet tensile, M.D. (p.p.i.) | 4                                            | 8              |
| Taber stiffness, M.D.      | 18.7                                         | 22.2           |
| Taber stiffness, C.D.      | 8.9                                          | 13.4           |
| Porosity (sec.)            | 88                                           | 56             |
| M.I.T. fold, M.D.          | 324                                          | 290            |
| M.I.T. fold, C.D.          | 502                                          | 532            |
|                            |                                              | 1,049          |

The following Table III represents a compilation of comparative average data computed for a plurality of experiments which were run with various resin and curing agent combinations. The table presents comparative data demonstrating the superior results obtained with high

45 Example (b) demonstrates a high level of bonding shown by increases in dry tensile, mullen, stiffness, and wet tensile. Vinylcyclohexene dioxide in the proper application of this method can be valuable in obtaining stiffness in paper.

Example (c) shows the same level of improvement in wet properties as Example (b) with lower levels of addition of epoxy.

50 Example (d) shows that higher amounts of CY179 is needed to equal the wet and dry properties of the previous examples but the sheet is more flexible. This method may be of use where strength and flexibility are desired.

Example (e) demonstrates a lack of an integrated cure 55 since the dry strength of the sheet was drastically impaired and no gain in wet strength was evidenced.

Example (f) shows a slight gain in dry physical properties and a slight gain in wet properties. This example illustrates the results obtained when a resin is cured in a sheet 60 without one of the reactants being bound to the cellulose before the reaction begins. A comparison of the results obtained in this example with those obtained in examples (b) and (c) in the following table will show the advantages of this invention.

65 Example (g) demonstrates improvements in tensile, stiffness and mullen can be achieved although the sequence of application of resin and curing agent is reversed.

Example (h) is a control to which no resin has been 70 added. In Table III the expression "RD2" represents 1,4-butanediol diglycidyl ether; the expression "RD4" represents vinylcyclohexenedioxide; the expression "CY179" represents alicyclic diepoxy carboxylate and the expression "Tandex 12" represents polyethyleneimine having a molecular weight from 40,000 to 60,000.

TABLE III

| Example  | Reactants                            | Percent of epoxy, (range) | Percent of amine, (range) | AV tensile, MD | AV tensile, CD | AV wet tensile, CD | AV percent wet tensile, CD | AV taber stiffness, MD+2CD | AV, Mullen |
|----------|--------------------------------------|---------------------------|---------------------------|----------------|----------------|--------------------|----------------------------|----------------------------|------------|
| (a)..... | Tydex 12.....                        | { 1-6                     | 50                        | 28             | 6.8            | 24                 | 35                         | 72                         |            |
|          |                                      | { 6-11                    | 50                        | 29             | 6.5            | 22                 | 35                         | 76                         |            |
| (b)..... | Tydex 12+RD4.....                    | { 16-20                   | 1-4                       | 57             | 32             | 13.0               | 40                         | 39                         | 87         |
|          |                                      | { 3-4                     | 58                        | 31             | 13.0           | 42                 | 42                         | 79                         |            |
| (c)..... | Tydex 12+RD2.....                    | { 10-13                   | 3                         | 45             | 28             | 14.0               | 50                         | 32                         | 83         |
|          |                                      | { 15-19                   | 3                         | 49             | 28             | 12.0               | 43                         | 33                         | 81         |
| (d)..... | Tydex 12+CY179.....                  | { 12-21                   | 2-4                       | 44             | 24             | 7.5                | 32                         | 28                         | 72         |
|          |                                      | { 32-37                   | 3-5                       | 57             | 31             | 12.5               | 40                         | 32                         | 81         |
| (e)..... | Triethylene tetraamine+RD4.....      | { 16-18                   | 5-6                       | 21             | 12             | 0.5                | 2                          | 34                         | 22         |
|          |                                      | { 19-23                   | 5-6                       | 20             | 11             | 0.5                | 2                          | 33                         | 18         |
| (f)..... | Triethylene tetraamine+RD2.....      | { 21-23                   | 5-6                       | 39             | 24             | 9.5                | 40                         | 32                         | 56         |
|          |                                      | { 28-37                   | 5-6                       | 29             | 19             | 6.8                | 36                         | 25                         | 43         |
| (g)..... | Tydex 12+RD2.....                    |                           | NA                        | 60             | 39             | NA                 | NA                         | 40                         | 116        |
| (h)..... | Control paper with no additives..... | (0)                       | (0)                       | 49             | 25             | 0.8                | 3                          | 31                         | 60         |

Delamination tests were run using a conventional Scott Bond Tester. Results of these tests indicate the internal strength of the paper sheet. In this test the lower the reading the lower the delamination resistance of the paper being tested. A commercial tabulating cardstock which was not resin treated produced a reading of 66.4 gram centimeters at rupture, and a commercial epoxy-impregnated card stock produced by a process such as that described in U.S. Pat. No. 3,131,083 produced a reading of 238 in the same test. Card stock produced in accordance with the conditions of Example XII was not delaminated at a reading of 500, the maximum reading possible on that machine.

In a different test to measure delamination resistance and consequently strength of internal fiber bond a standard commercial untreated card stock produced a 7.5 ounce-inch reading, a commercial epoxy impregnated card stock produced by a process such as that described in U.S. Pat. No. 3,131,083 produced a 12.5 reading and the card stock of Example XII produced a 25.5 reading.

What is claimed is:

1. A modified cellulosic material derived from a mixture of (a) a fibrous cellulosic material and (b) about 0.1 to about 10 weight percent, based on the dry weight of (a), of cellulose-substantive polyethyleneimine having a molecular weight between about 500 and 100,000; said mixture impregnated and reacted substantially throughout said fibrous material with an aqueous dispersion of (c), a polymerizable unreacted epoxy resin having a molecular weight up to about 1,000.

2. A process for producing an epoxy-modified paper on a paper machine comprising the steps of: (a) adding to the papermaking furnish about 0.1 to about 3 weight percent, based on the weight of cellulosic pulp material in such furnish, of cellulose-substantive polyethyleneimine having a molecular weight between about 500 and 100,000; (b) forming a web from such treated furnish; (c) intimately contacting such formed paper web with an aqueous dispersion comprising from about 0.1 to 30 weight percent, based on the weight of pulp in such furnish, of an unreacted epoxy resin having a molecular weight up to about 1,000; and (d) heating the epoxy-containing web to permit substantial cure thereof on the paper machine.

3. A process as set forth in claim 2, wherein said epoxy dispersion is applied from a size press, and the viscosity of said aqueous dispersion is less than about 100 centipoises.

4. A process as set forth in claim 2, wherein said aqueous dispersion includes about 2% by weight of

1,4-butanediol diglycidyl ether and about 2% by weight of a bisphenol A-epichlorohydrin resin having a molecular weight of about 400.

5. A process as set forth in claim 2, wherein said aqueous dispersion includes an amount in the range from about 5 to about 20% by weight of starch.

6. A process as set forth in claim 2, wherein said heating occurs at a temperature in the range from about 170° F. to about 300° F.

7. A process as set forth in claim 2, wherein said furnish has a pH in excess of 7.

8. A modified cellulosic sheet material as defined in claim 1 wherein component (c) is a mixture of 1,4-butanediol diglycidyl ether and the condensation product of bisphenol A and epichlorohydrin.

9. A composition as defined in claim 1 wherein component (b) is present in the amount of from about 0.1 to about 3 weight percent, based upon the dry weight of the cellulosic fibrous material.

10. A composition as defined in claim 1 wherein the unreacted epoxy resin has a molecular weight of up to about 500.

11. A composition as defined in claim 1 wherein the viscosity of the aqueous dispersion is no more than about 100 centipoises at 25° C.

12. A composition as defined in claim 1 wherein the unreacted epoxy resin is present in the amount of from about 0.1 to about 30 weight percent, based on the total weight of the aqueous dispersion.

13. A composition as defined in claim 1 wherein the unreacted epoxy resin is present in the amount of from about 2 to about 12 weight percent, based on the total weight of the aqueous dispersion.

#### References Cited

##### UNITED STATES PATENTS

|           |         |            |       |            |
|-----------|---------|------------|-------|------------|
| 2,913,356 | 11/1959 | Schroeder  | ----- | 162—164    |
| 3,250,665 | 5/1966  | Goss       | ----- | 162—182    |
| 3,257,342 | 6/1966  | Kwong      | ----- | 260—47EPCN |
| 3,378,434 | 4/1968  | Harrington | ----- | 260—830TW  |
| 3,381,053 | 4/1968  | Vogt       | ----- | 260—830TW  |
| 3,291,775 | 12/1966 | Holm       | ----- | 260—47EPCN |
| 3,418,204 | 12/1968 | Goldstein  | ----- | 162—164    |

S. LEON BASHORE, Primary Examiner

R. H. ANDERSON, Assistant Examiner

U.S. Cl. X.R.

8—116.2; 162—166, 169, 182, 185; 260—2 EN, 47EP